

1

2,977,224

## COBALT-BASE ALLOY

William H. Faulkner, Kokomo, Ind., assignor to Union Carbide Corporation, a corporation of New York

No Drawing. Filed Dec. 4, 1958, Ser. No. 778,053

3 Claims. (Cl. 75—171)

This invention relates to a cobalt-base alloy for high temperature service and, more particularly, to a cobalt-base alloy suitable for high temperature service in either cast or wrought form.

Research directed to increasing the power and efficiency of jet propulsion and gas turbine engines have provided designs for engines that will operate at higher temperatures than currently known metals and alloys can withstand. Metals and alloys capable of withstanding these high-temperature stresses are avidly sought therefore. Furthermore, alloys are sought which, in addition to possessing outstanding high-temperature strength, must also be capable of being fabricated into useful parts by known methods.

In some cases the alloys may be employed in the form of castings, while for other operations these alloys must be capable of being hot-worked into sheet and strip, or subjected to cold-working or machining. Furthermore, materials fabricated from these alloys must have good oxidation, impact and thermal shock resistance.

While several alloys have been proposed for high temperature service under the conditions set forth above, none have possessed the required combination of high strength, high heat resistance and high workability.

The primary object of this invention, therefore, is to provide an alloy which has higher tensile, stress-rupture, and impact resistance than alloys heretofore known, as well as increased ductility and creep-rupture strength, to enable its use in a wide variety of applications at temperatures higher than the limiting temperatures of currently known alloys and up to a temperature of about 1800° F.

Another object of this invention is to provide an alloy with high oxidation resistance and fatigue strength at elevated temperatures.

A further object of the invention is to provide an alloy suitable for use at elevated temperatures which may be fabricated by casting or forging, and which can be cold-worked to increase its hardness.

Other aims and advantages of the invention will be apparent from the following description and appended claims.

In accordance with the present invention, a cobalt-base alloy is provided having compositions defined by the ranges given in Table A.

TABLE A

| Constituent: | Percentage by weight |
|--------------|----------------------|
| Chromium     | 19 to 22             |
| Tungsten     | 11.5 to 13.5         |
| Molybdenum   | Up to 3              |
| Iron         | Up to 3              |
| Carbon       | Less than 0.25       |
| Cobalt       | Balance              |
| Nickel       | Up to 1              |
| Boron        | Less than 0.15       |
| Nitrogen     | Up to 0.06           |
| Silicon      | Up to 1              |
| Manganese    | Up to 1              |

2

In a preferred embodiment of this invention, the alloy consists essentially of about 20 percent by weight chromium, about 12.5 percent by weight tungsten, about 0.15 percent by weight carbon, up to about 0.03 percent by weight boron, up to about 0.03 percent by weight nitrogen, and the balance being substantially all cobalt.

Chromium and tungsten both improve the high temperature strength of the alloy, and give the alloy increased ability to resist deformation while under severe loading. Tungsten may be complemented by molybdenum in amounts up to 3 percent by weight molybdenum. The addition of molybdenum will increase high temperature tensile and stress-rupture strength at the expense of a loss of room temperature ductility. Therefore, the molybdenum content is limited to 3 percent.

While the presence of nickel increases toughness at lower temperatures it causes a reduction in high temperature strength. Therefore the nickel content should be adjusted to achieve specific desired results. For high temperature service the nickel content should not be greater than one percent.

Carbon and boron are necessary additions for ductility and strength in products composed of this alloy. Although the addition of boron greatly increases the strength of this alloy, boron is detrimental to oxidation resistance, and therefore the desired level of boron content is dependent upon the anticipated service temperature of the alloy. The boron content is of critical importance and must carefully controlled as indicated below. However, while higher carbon contents are suitable for casting operations, when the alloy is to be rolled both the carbon and boron contents should be lowered.

The high temperature strength of the cobalt matrix is further increased by the existence of a precipitated-phase, composed of carbides of the  $M_6C$  type, where "M" refers to the carbide formers cobalt, chromium, tungsten and molybdenum. Of especial importance are the rates of diffusion of chromium and carbon in the cobalt-rich matrix. If these elements are able to diffuse rapidly through the matrix, the carbides are readily formed and grow rapidly yielding a hardening through precipitation. However, beyond a limiting size and concentration, these carbides are no longer useful in increasing the strength of the alloy. Therefore by limiting the diffusion of carbon and chromium, the rate of growth of these carbides is diminished and their size kept within limits with the desired result that the alloy achieves maximum strength from this precipitate hardening phase. Tungsten, chromium, and nickel are effective in controlling the diffusion of carbon and the formation of carbides.

Manganese and silicon may be present in amounts up to 1 percent by weight of each. These elements are found as impurities in the constituents of the alloy and are useful as deoxidizers.

Iron may be present in amounts up to 3 percent; but since iron does not contribute to high temperature strength, it should be limited to amounts not exceeding one percent in the preferred alloy composition.

The amount of nitrogen in the alloy is of critical importance. Heretofore it was thought that nitrogen was essential in alloys of this type, but it has been found to have a deleterious effect on cobalt-base alloys. Table B clearly indicates the effect of nitrogen on a cobalt-base alloy of this type.

**3**  
**TABLE B**  
*Stress-rupture data at 1700° F. and 20,000 p.s.i.*

| Nitrogen content, percent by weight | Life, Hours | Elongation, Percent | 10 |
|-------------------------------------|-------------|---------------------|----|
| 0.03                                | 94.7        | 16                  |    |
| 0.06                                | 30.5        | 18                  |    |
| 0.07                                | 21.7        | 14                  |    |
| 0.08                                | 22.0        | 5                   |    |
| 0.09                                | 18.4        | 17                  |    |

Therefore the nitrogen content should be kept below 0.06 percent by weight, and preferably below 0.04 percent for maximum strength in the alloy.

The alloy may be melted by standard furnacing procedures, such as by induction heating, and should be conducted in the protective atmosphere of an inert gas, such as argon. This shielding of the molten metal by an inert gas will prevent contamination by the nitrogen in the air. The alloy may be used in the as-cast condition.

This alloy may also be fabricated by hot or cold working into useful parts. When ingots are required for forging, the melting is preferably conducted under vacuum conditions. By maintaining the carbon content below about 0.20 percent by weight and the boron content below about 0.15 percent by weight, the alloy can be mechanically fabricated by known methods to produce such items as wire, strip, rod, plate, bar, sheet, tubings, forgings, and extruded shapes. These products all have excellent mechanical properties at elevated temperatures. The alloy may also be rolled into sheets. Table C gives typical stress-rupture data for sheet products having the following composition by weight: 20 percent chromium, 12.5 percent tungsten, 0.15 percent carbon, 0.028 percent boron, 0.01 percent nitrogen, and the balance substantially all cobalt.

**TABLE C**  
*Stress-rupture data for 0.109 inch thick sheet*

| Temperature, ° F. | Stress, p.s.i. | Life, Hours | Elongation, Percent |
|-------------------|----------------|-------------|---------------------|
| 1,700             | 15,000         | 216.7       | 18                  |
| 1,700             | 13,000         | 397.3       | 29                  |
| 1,800             | 10,000         | 75.2        | 25                  |
| 1,800             | 8,000          | 294.4       | 23                  |

In another example of the invention, an alloy having a composition of about 19.98 percent chromium, about 12.35 percent tungsten, about 0.06 percent carbon, about 0.005 percent boron, about 0.48 percent silicon, about 0.48 percent manganese, and the balance substantially all cobalt was fabricated into sheet products which had the stress-rupture strengths shown in Table D.

**TABLE D**  
*Stress-rupture data for 0.040 inch thick sheet*

| Temperature, ° F. | Stress, p.s.i. | Life, Hours | Elongation, Percent |
|-------------------|----------------|-------------|---------------------|
| 1,500             | 30,000         | 59.6        | 43                  |
| 1,600             | 24,000         | 47.3        | 73                  |
| 1,700             | 15,000         | 93.8        | 77                  |
| 1,800             | 10,000         | 49.3        | 38                  |

The results shown in Tables C and D demonstrate the high stress-rupture properties of the alloys of this invention. These superior properties are due to the critical compositions shown. The constituents must be present in the proportions disclosed herein if the highest strengths are to be achieved. Of especial importance are the low nitrogen content of these alloys and the careful control of the boron content.

In the wrought form, the alloy has sufficient ductility to permit cold-working, and as a result of such cold-

working, the hardness of the alloy increases considerably as seen in Table E. Additionally the hardness may be further increased by subjecting the cold-worked alloy to heat-treatments. The increase in hardness may be obtained by heat-treating at temperatures as low as 1200° F. The use of a comparatively low temperature age-hardening heat treatment is particularly significant for the low temperatures guarantee a minimum of distortion in finished parts.

**TABLE E**  
*Hardness of sheet products*

| Gage, Inch | Cold Reduction, Percent | Hardness as Cold-Rolled, Rockwell C Test | Hardness After Aging, Rockwell C Test |
|------------|-------------------------|------------------------------------------|---------------------------------------|
| 0.036      | 20                      | 46                                       | 52                                    |
| 0.063      | 20                      | 49                                       | 53.5                                  |
| 0.090      | 25                      | 51                                       | 55.5                                  |

Because of its unique properties in the cold-worked form, the alloy has a special usefulness in applications requiring high hardness for wear- and abrasion-resistance.

The alloys of this invention also show a remarkable improvement in tensile properties while still possessing sufficient ductility for a wide variety of uses. Table F demonstrates the outstanding tensile strength-ductility relationship of any alloy having the same composition as that used in the tests of Table D.

**TABLE F**  
*Tensile test data for 0.040 inch thick sheet*

| Temperature, ° F. | Ultimate Strength, p.s.i. | Yield Strength, 0.2% Offset, p.s.i. | Elongation, Percent |
|-------------------|---------------------------|-------------------------------------|---------------------|
| Room              | 164,000                   | 82,500                              | 37                  |
| 1,200             | 119,500                   | 53,800                              | 20                  |
| 1,400             | 96,800                    | 52,300                              | 24                  |
| 1,600             | 53,300                    | 39,800                              | 45                  |

<sup>1</sup> Bar stock.

High impact strength is required in many applications. Table G shows the outstanding results of impact strength tests conducted on alloy specimens having the following composition: 19.98 percent chromium, 12.35 percent tungsten, 0.16 percent carbon, 0.005 percent boron, 0.48 percent silicon, 0.72 percent manganese, and the balance substantially all cobalt. The alloy was tested in the annealed condition with a 30 minute heat treatment at 2125° F. followed by a rapid air cool.

**TABLE G**  
*Impact strength data*

| Temperature, ° F. | Average Charpy V-Notch Impact Strength, ft.-lbs. |
|-------------------|--------------------------------------------------|
| Room              | 72                                               |
| 1,200             | 104                                              |
| 1,350             | 101                                              |
| 1,500             | 97                                               |
| 1,600             | 98                                               |
| 1,700             | 92                                               |

What is claimed is:

1. A cobalt-base alloy consisting essentially of from 19 to 22 percent by weight chromium, from 11.5 to 13.5 percent by weight tungsten, up to 3 percent by weight molybdenum, up to 3 percent by weight iron, up to 1 percent by weight nickel, up to 0.25 percent by weight carbon, up to 0.15 percent by weight boron, up to 0.06 percent by weight nitrogen, manganese and silicon in amounts up to 1 percent by weight of each, and the balance substantially all cobalt.

2. A cobalt-base alloy consisting essentially of about 20 percent by weight chromium, about 12.5 percent by weight tungsten, about 0.15 percent by weight carbon, up to about 0.03 percent by weight boron, up to about 0.04 percent by weight nitrogen, less than 1 percent by weight each of manganese and silicon, and the balance substantially all cobalt.

3. A cobalt-base alloy consisting essentially of about

20 percent by weight chromium, about 12.35 percent by weight tungsten, about 0.16 percent by weight carbon, about 0.005 percent by weight boron, about 0.48 percent by weight silicon, about 0.72 percent by weight manganese, and the balance substantially all cobalt.

References Cited in the file of this patent

Woldman et al.: "Engineering Alloys," published by ASM (1936), pages 138 and 238 relied on.